

## UNITED STATES PATENT OFFICE.

ANDREW G. COLLIAS, OF DETROIT, MICHIGAN.

## COMPOSITION FOR WHITE SHOE DRESSING.

No Drawing.

Application filed December 29, 1923. Serial No. 683,371.

*To all whom it may concern:*

Be it known that I, ANDREW G. COLLIAS, a citizen of the United States, residing in the city of Detroit, county of Wayne, State 5 of Michigan, have invented certain new and useful Improvements in a Composition for White Shoe Dressing, of which the following is a specification.

My invention relates to a composition of 10 liquid and powdered ingredients, mixed together and compounded into a liquid dressing for shoes.

The object of my invention is to provide a white dressing for shoes, of high 15 grade, and possessing great adhesive qualities when applied to the surface of the shoe.

A further object is to produce a dressing that dries quickly and leaves the surface of the shoe perfectly white and without streaking, or injuring the material to which it 20 is applied.

Another object is to produce a white dressing that can be applied to either leather or cloth shoes, easily and efficiently and can 25 be manufactured at a low cost.

In compounding the ingredients for the dressing, the inventor has used such materials that will preserve, adhere to, and re-surface the shoe when applied thereto, using 30 oils for softening the leather, if applied to a leather shoe, an adhesive liquid, and coloring powders for producing a pure white color when dried on the surface of the shoe. For softening and preserving the leather, a 35 composition of oil of bitter almond and oil of citronella is used, being mixed with a powdered composition of light zinc oxide, magnesium carbonate and purified talcum, for producing the white coloring matter and 40 forming a body for the dressing. A small quantity of beeswax may also be added to give luster and hardness to the surface when dried, and the composition being made adhesive by adding thereto a very small quantity of stearic acid. A quantity of pure gasoline and carbon tetrachloride is then added to 45 for the purpose of cleaning and absorbing particles on the leather surface, and for drying quickly when the dressing is applied.

In preparing the composition, I prefer to

use the following proportions of the ingredients:

|                      |           |    |
|----------------------|-----------|----|
| Oil of bitter almond | 2 dr.     |    |
| Oil of citronella    | 2 dr.     | 55 |
| Stearic acid         | 1/2 oz.   |    |
| Light zinc oxide     | 16 oz.    |    |
| Magnesium carbonate  | 16 oz.    |    |
| Purified talcum      | 32 oz.    |    |
| High test gasoline   | 1 gal.    |    |
| Carbon tetrachloride | 1 qt.     |    |
| Beeswax              | 1 1/2 oz. |    |

With the above proportions of the ingredients, the best results are obtained, and the dressing is easily applied to the surface of the shoe, and is dried and polished in the ordinary manner. It is understood that while I have stated only the preferred proportions of ingredients used in my white dressing, it is obvious that my invention is 65 capable of various modifications in proportions, and without departing from the spirit of my invention. Very good results may be obtained by varying the various ingredients used in compounding the dressing, between 70 75 the following limits:

|                      |                       |    |
|----------------------|-----------------------|----|
| Oil of bitter almond | from 1 dr. to 3 dr.   |    |
| Oil of citronella    | from 1 dr. to 3 dr.   |    |
| Stearic acid         | from 1/4 oz. to 1 oz. | 80 |
| Light zinc oxide     | from 12 oz. to 20 oz. |    |
| Magnesium carbonate  | from 12 oz. to 20 oz. |    |
| Purified talcum      | from 20 oz. to 40 oz. |    |
| High test gasoline   | from 3 qt. to 5 qt.   |    |
| Carbon tetrachloride | from 1 pt. to 3 pts.  | 85 |
| Beeswax              | from 1 oz. to 3 oz.   |    |

It is understood that the preferred formula as set forth, is not confined to the specific quantities therein named for each ingredient, but such quantities only represent a 90 relative proportion of each ingredient used.

In compounding my white shoe dressing, either one of the oil ingredients may be omitted, for the purpose of decreasing the cost, also the magnesium carbonate may be 95 omitted, although the quality of the dressing will be greatly reduced, and not producing the results as are obtainable with the proportions set forth in the preferred formula.

Having fully described my white shoe dressing, what I claim as my invention and desire to secure by Letters Patent is:

1. A composition adapted for dressing and polishing white shoes, comprising the following ingredients in the proportions named; oil of bitter almond, 2 drams; oil of citronella, 2 drams; stearic acid,  $\frac{1}{2}$  ounce; zinc oxide, 16 ounces; magnesium carbonate, 16 ounces; talcum, 32 ounces; carbon tetrachloride 1 quart; beeswax,  $1\frac{1}{2}$  ounces; gasoline, one gallon; all thoroughly mixed together and compounded into a liquid form.
2. A composition of matter adapted as a white dressing and polish for shoes comprising oil of bitter almond from one to three drams; oil of citronella from one to three drams; stearic acid from one fourth to one ounce; light zinc oxide from twelve to

twenty ounces; magnesium carbonate from 20 twelve to twenty ounces, talcum twenty to forty ounces; carbon tetrachloride from one to three pints; beeswax from one to three ounces; gasoline from three to five quarts, all thoroughly mixed together in a liquid 25 form.

3. A composition of matter adapted for use as white dressing for shoes, comprising oil of bitter almond 1 to 3 drams; stearic acid  $\frac{1}{4}$  to 1 ounce; zinc oxid 12 to 20 ounces; magnesium carbonate 12 to 20 ounces; talcum 20 to 40 ounces; carbon tetrachloride 1 to 3 pints; beeswax 1 to 3 ounces; gasoline 1 to 5 quarts; all mixed together and compounded in a liquid form.

In witness whereof I sign these specifications.

ANDREW G. COLLIAS.